

## UNITED STATES PATENT OFFICE.

EDWARD HENRY NOACK, OF STOCKTON, CALIFORNIA.

## HEAT-RESISTING STEEL.

No Drawing.

Application filed June 14, 1924. Serial No. 720,122.

*To all whom it may concern:*

Be it known that I, EDWARD H. NOACK, a citizen of the United States, residing at Stockton, county of San Joaquin, State of California, have invented certain new and useful Improvements in Heat-Resisting Steel; and I do declare the following to be a full, clear, and exact description of the same.

10 This invention relates to the metallurgical art, and particularly to steel making; my principal object being to produce a steel of a heat resisting nature, suitable for any purpose where the metal is subjected to 15 high temperatures when in service. This steel is especially adapted for making grate-bars; fire-door liners, arches and bearing bars; case hardening carbonizing pots; gas engine valves; oil valves, and in fact any 20 place where the conditions of operation require a heat resisting metal.

The improved steel contains, besides the main body of iron, silicon, manganese, carbon, sulphur, phosphorus, and copper, 25 These alloying elements are combined in the following proportions in the finished product:

30 Silicon, 1.50 to 2.00%; copper, 0.50 to 1.00%; manganese, 0.12% and under; carbon, 0.10% and under; sulphur, .06% and under; phosphorus, .06% and under.

It will be noted from the above formula 35 that the silicon and copper content is very high compared to the other elements, particularly with regard to the manganese and carbon. The high silicon and copper content, and the low manganese and carbon content, are the factors which together control the heat resisting properties of the steel. 40 The high content of the two first named elements is necessary to impart the desired heat resisting qualities to the steel, while

a low manganese and carbon content is also necessary in obtaining this result.

In other words steel with a high silicon 45 and copper content, with an equally high manganese and carbon content, would not have the desired properties, and neither would a steel having a low manganese and carbon content and a proportionately low 50 silicon and copper content.

In practice, I preferably prepare the special steel from ordinary scrap steel, which usually contains all the above elements except copper. An analysis of such steel usually discloses however that silicon is not present in sufficient quantity, while there is 55 too much manganese and carbon.

The particular phosphorus and sulphur content is not especially vital to my product, and do not interfere with the heat resisting properties to be obtained. The proportions of these elements is usually such that they may be left undisturbed.

The manganese and carbon content is 65 therefore reduced to the desired amount, by methods well known to the steel maker, and the requisite amount of silicon and copper added. The exact proportion of manganese may be varied somewhat according to the 70 strength desired in the final product.

This metal, with the exception that the copper is omitted, is also highly suitable for lead pots and cyanide hardening pots.

Having thus described my invention 75 what I claim as new and useful and desire to secure by Letters Patent is:

A steel containing silicon between 1.50% and approximately 2.00%; copper between 0.50% and approximately 1.00%; manganese not over 0.12%; and carbon not over 0.10%.

In testimony whereof I affix my signature.  
EDWARD HENRY NOACK.